

# UNITED STATES PATENT OFFICE.

RICHARD SMITH WILLOWS, OF MANCHESTER, FREDERICK TOMLINSON POLLITT, OF WORSLEY, AND THOMAS LEACH, OF MANCHESTER, ENGLAND.

## PRODUCTION OF PATTERN EFFECTS IN COTTON AND OTHER VEGETABLE FIBER FABRICS, ALSO INCLUDING SILK.

1,411,598.

Specification of Letters Patent. Patented Apr. 4, 1922.

No Drawing.

Application filed January 11, 1922. Serial No. 528,578.

To all whom it may concern:

Be it known that we, RICHARD SMITH WILLOWS, FREDERICK TOMLINSON POLLITT, and THOMAS LEACH, subjects of the King of Great Britain, residing at Manchester, Worsley, and Manchester, all in the county of Lancaster and Kingdom of England, have invented certain new and useful Improvements in the Production of Pattern Effects in Cotton and other Vegetable Fiber Fabrics, also Including Silk, of which the following is a specification.

The present invention relates to improvements in the production of pattern effects on cotton and other vegetable fiber fabrics and also including silk hereafter termed textile organic fabrics.

The object of the invention is to obtain certain delicate yet clearly defined effects.

It is of course common to produce pattern effects by embossing fabrics either in the dyed or undyed or mercerized or unmercerized condition by subjecting the fabric to the action of suitable embossing means, usually a heated roller upon which there is a pattern in relief. In view of the fact that subsequent treatment with water is capable of partially or completely nullifying the effect of the embossing which appears to be either in the direction of compression of the fiber or change of its state of hydration, it was to be expected that the delicacy of such patterns would be seriously impaired if not destroyed by subjecting embossed fabrics to the action of dyeing solutions.

It has in fact been proposed to mercerize a fabric and to emboss this fabric while in the wet state and thereupon to dye the embossed fabric. Study of this proposal in practice demonstrates however that the edges of the pattern are blurred and that the desired delicate and sharply defined pattern cannot be obtained in this way; it may be noticed that this proposal only extended to mercerized materials and not to unmercerized materials.

It is the object of the present invention to overcome this disadvantage and this result has been successfully achieved by employing the following steps in combination, viz:

(1) Conditioning the fabric so that it contains from about 5 to 15% of water, i. e. fabric containing the amount of water common to air-dry or slightly moist condition.

This conditioning may be performed either 55 by damping the dry fabric or by drying the damp fabric or by selecting the fabric at the right stage of dryness. (This amount of moisture is critical since if "wet" fabrics are used, blurred effects are obtained.) 60

(2) Embossing a pattern on the conditioned fabric by suitable embossing means.

(3) Subjecting the embossed fabric to treatment by a dyeing or a mercerizing or parchmentizing agent, either single or in 65 combination.

These three steps are essential and if they are all applied it will be found that a delicate yet well-defined pattern will be obtained on the dyed or mercerized or parchmentized 70 fabric. If uniform compression is used, a uniform sheen is imparted to the fabric after step 3.

Thus a fabric of cotton or other vegetable fiber, flax, jute, ramie or nettle, or also a 75 fabric of silk may or may not be treated with any of the usual processes preparatory to dyeing such as scouring, bleaching, mordanting, crêping or mercerizing or parchmentizing and is then damped or dried until it 80 contains 7-15% of water as determined by drying for one hour at a temperature of 212° F.

The conditioned fabric is then pressed, e. g. under a heated embossing roller or plate 85 bearing the desired pattern or design in relief.

The embossed fabric is then dyed and may be finished by any of the usual processes 90 incidental to this operation for instance calendering, printing, embossing, mercerizing, schreinering or raising. In some cases the dying may be replaced by operation such as mercerizing or parchmentizing. The essential point of this third step is that the 95 fabric is treated with some reagent whereby a differential effect is produced so that a pattern results. In other words, we can cause fixation of the pattern by the use of a suitable chemical reagent such as the dye or 100 parchmentizing agent or other agents. By parchmentizing after embossing, plain cotton fabrics may be caused to resemble brocade. The designs or patterns so produced are not only clearly defined when 105 made but remain clearly defined through all processes to which the fabrics are likely to be submitted in laundering, or other cleaning

processes to which the fabric or articles made therefrom are likely to be submitted in or after use.

The fabrics prepared as described are characterized by the feature that although the relief caused by embossing has disappeared, i. e. the pattern is in one plane, yet the moisture content per unit area is different in the parts of the fabric forming the pattern and the background. This difference is due to the application of pressure and heat during embossing and it persists after the further treatment described.

We declare that what we claim is:

15. 1. The process of treating textile organic fabrics which comprises compressing a fabric containing from 5% to 15% of moisture and then subjecting the compressed fabric to the action of a chemical reagent.
20. 2. The process of treating a textile organic fabric which comprises conditioning the fabric till it contains 5% to 15% of moisture, compressing the fabric and then subjecting the fabric to the action of a chemical reagent which has a different action on compressed and uncompressed fabric.
25. 3. The process of treating cotton fabric which consists in compressing fabric containing 5% to 15% of moisture and submitting the compressed fabric to the action of a chemical reagent.
30. 4. The process of treating a textile organic fabric which comprises embossing the fabric containing 5% to 15% of moisture to produce a pattern, and then treating the embossed fabric with a chemical reagent to make the pattern permanent.
35. 5. The process of treating unmercerized

cotton fabric which comprises compressing the fabric and then submitting the compressed fabric to the action of a chemical reagent.

6. The process of treating unmercerized cotton fabric which comprises embossing a pattern thereon and then treating the fabric with a chemical reagent to make the pattern permanent.

7. The process of treating a cotton fabric which comprises embossing a fabric containing 5% to 15% of moisture, and then treating the embossed fabric with a parchmentizing reagent.

8. Textile organic fabrics having a delicate yet clearly defined pattern produced by embossing the fabric containing 5% to 15% of moisture and made permanent by action of a chemical reagent.

9. A cotton fabric having a delicate yet clearly defined pattern produced by embossing the fabric containing 5% to 15% of moisture and made permanent by action of a chemical reagent.

10. A textile organic fabric having its surface modified by compression of the fabric containing 5% to 15% of moisture followed by fixation with a chemical reagent.

In witness whereof, we have hereunto signed our names this 23rd day of December 1921, in the presence of two subscribing witnesses.

RICHARD SMITH WILLOWS.  
FREDERICK TOMLINSON POLLITT.  
THOMAS LEACH.

Witnesses:

JOHN WILLIAM THOMAS,  
ERNALD S. MOSELEY.